

July 1, 1930.

R. D. PIKE

1,769,604

## METALLURGICAL PROCESS

Original Filed Sept. 23, 1925

*Fig. I.*



Fig. 2.



## UNITED STATES PATENT OFFICE

ROBERT D. PIKE, OF PIEDMONT, CALIFORNIA

## METALLURGICAL PROCESS

Application filed September 23, 1925, Serial No. 58,012. Renewed February 27, 1928.

This invention relates to a process for recovery of metals from a wide variety of ores and concentrates with production of electrolytic iron. It has been demonstrated that 5 metals are dissolved from sulphide minerals to a greater or lesser extent by solutions containing ferric salts such as a chloride or sulphate, with the consequent reduction of the ferric salt to the corresponding ferrous salt 10 and the precipitation of elemental sulphur; and that the ferrous solutions can be treated in a diaphragm electrolytic cell for the regeneration of the ferric salt and the consequent deposition of electrolytic iron. However, up to the present time, unsolved difficulties have prevented the successful commercial application of a process of the above general description.

The first of these unsolved difficulties is the 20 sluggishness of the ferric solutions as solvents. Some few sulphide minerals are attacked with fair rapidity and completeness, while others are attacked but slowly and incompletely. All results of work to date, including my own, show that with all sulphide minerals ferric chloride is a more active solvent than ferric sulphate, but that the former is not, in most cases, active enough to be considered of itself, alone, a satisfactory commercial 25 solvent for many important sulphide minerals, such, for example, as chalcopyrite. On this account, and because ferrous chloride is a more satisfactory electrolyte in the electrolytic iron cell, the chloride is to be preferred over the sulfate, and my present process is particularly adapted to the use of a chloride leach and electrolyte, but can also be used, if desired, with a sulfate leach. The 30 superiority of the chloride leach and electrolyte over the sulphate for the stated reasons is well-known, and presents the second unsolved difficulty; namely, a cheap means for maintaining a ferric-ferrous chloride cycle of this type. The difficulty arises from 35 the fact that certain compounds of magnesia, alumina, and lime, which occur in many ores and concentrates, are very soluble in ferric chloride; and the only way to keep the concentration of such compounds (and possibly 40 others) within allowable limits, is to discard

a portion of the electrolyte at each cycle, involving a loss of costly chlorine.

My present invention has for its object to obtain substantially complete extraction from, and recovery of, metallic values from 55 a wide variety of sulphide ores and concentrates in a cyclic process which produces pure electrolytic iron and elemental sulphur as by-products; and to cheaply maintain in standard condition the ferric-ferrous chloride 60 leach-electrolyte used in the process.

In the following description and accompanying drawings I disclose a conventional type of electrolytic cell for converting the ferrous chloride to ferric chloride and depositing electrolytic iron. In my prior Patent number 1,689,597, issued October 30, 1928, and entitled "Cell for electro-deposition of metals," filed concurrently herewith, there is disclosed a method and means for overcoming the other principal unsolved difficulty above referred to, namely, the successful large-scale deposition of electrolytic iron 65 from leach solutions.

Having outlined the general object of my invention, I will describe, by way of example but not for limitation, its application to a certain chalcopyrite copper concentrate of the following analysis:

|         |       |                                |      |        |          |    |
|---------|-------|--------------------------------|------|--------|----------|----|
| Copper  | 23.25 | Al <sub>2</sub> O <sub>3</sub> | 1.70 | Insol. | 8.56     | 80 |
| Iron    | 30    | CaO                            | .49  | Silver | 6.95 oz. |    |
| Sulphur | 29.52 | MgO                            | .36  | Gold   | 25 oz.   |    |

In the accompanying drawings, Fig. 1 shows one form of flow sheet; and Fig. 2 shows a form providing an alternative in one part of the process.

The return anolyte leach from the electrolytic cells, containing about 12% iron (about one-half as ferrous chloride and one-half as ferric chloride), and at a temperature of 90 about 70° C., enters the agitator 1 in a continuous stream. Into the same agitator is fed a continuous stream of the concentrates. Live steam is introduced, to raise the temperature to 90° C. to 100° C. Agitation is preferably furnished by a rubber-covered propeller suspended in the usual manner, and not shown. The concentrates should be finely ground, so that not less than 95% is minus 95 200 mesh.

The agitator is so proportioned to the work in hand that the time of residence of the leach is about two hours. In this time and under the conditions stated, from 85% to 90% of the copper will be dissolved; 70% to 75% of the iron; 85% to 90% of the silver; and 15% to 20% of the gold; and corresponding amounts of elemental sulphur precipitated. The proportion of leach liquor to 10 concentrates is so chosen that the ferric iron content in the effluent is 1% to 1.5%. The effluent passes continuously into the second agitator 2 (similar to 1), where it is also heated by steam to 90% to 100%, and into 15 which is introduced a stream of finely-ground pyrrhotite, or distilled pyrite, equivalent in weight to about 15% of the original concentrates. The function of the pyrrhotite is to reduce the ferric iron content of the liquor to 20 .1% to .2% without at the same time reprecipitating any appreciable amount of the copper and silver; although the greater part of the gold, dissolved in agitator 1, is reprecipitated in agitator 2 by the pyrrhotite. 25 Most of the gold remains with the tails from the agitators, while most of the silver remains in solution.

The tails are now dewatered by any usual means illustrated conventionally as classifier 3, thickener 4, and filter 5. The solid residue, or so-called No. 1 tails, represents about half the original weight of concentrates, and contains 30% to 40% of elemental sulfur, together with sulphur in combination with the 35 undissolved metals. This residue may be treated in sulphur-distilling retorts 7, and the elemental sulphur recovered as refined sulfur in condenser 8. The residue from the retorts goes to roaster 9, where the metals are 40 partly sulfated and partly oxidized; or the sulphur-distilling retorts can be entirely omitted and all the free sulphur burned to  $\text{SO}_2$  in a roaster. If all the sulphur is burned to  $\text{SO}_2$  in the roaster, there remains, 45 after deducting the sulphur necessary for manufacturing acid, required in a later step of the process, about one pound of sulphur per pound of original copper in the form of  $\text{SO}_2$  for making surplus acid for sale. 50 Whether or not the sulphur-distilling retorts be used, the calcines from the roaster go to agitator 10, where they are treated with sulphuric acid and steam, which dissolves practically all of the copper, leaving a tail with 55 .2% copper, or less, and also dissolves 30% to 40% of the iron remaining undissolved after the first, or chloride leach. The amount of iron dissolved in this leach can be controlled at the will of the operator within limits by 60 varying one or all of the factors of time, temperature, and strength of acid. The copper is far more soluble than the iron, and if the roast be carried out carefully to produce a maximum amount of copper sulfate, practically all of the copper is rendered soluble 65

in water. Ordinarily, with the concentrates being considered, about .75 pounds of commercial sulphuric acid is required per pound of copper in the original concentrate.

The tails from the second, or sulfate leach, 70 are dewatered in the usual manner, conventionally illustrated by classifier 11, thickener 12, and filter 13. The tails are greatly reduced in weight as compared with the original concentrate, and as they contain 75 80% to 90% of the original gold and about 10% of the original silver, are virtually a precious-metal-concentrate, and can be treated 80 in any well-known manner for the recovery of these metals.

The liquor from the sulfate leach containing copper and ferric sulfates goes to agitator 14, where it is mixed with calcium chloride, the greater part of which comes from a subsequent step of the process, and the 85 smaller part of which is that amount necessary to supply chlorine which is lost in the leaching process. The reaction between the copper and ferric sulfates and the calcium chlorides precipitates artificial gypsum and 90 transforms the copper and iron respectively to cupric and ferric chlorides. The gypsum is dewatered and washed by any usual means, conventionally illustrated as thickener 15 and filter 16. The gypsum can easily be 95 washed free from copper and iron, and is a saleable by-product of which about one pound is produced per pound of copper in the original concentrates. The chloridized liquor from 14, together with that from agitator 1, or chloride leach, goes to copper cementation drum 6, or other suitable apparatus, for precipitating copper on iron. The cement copper is dewatered in 17, and goes 100 to a refinery. This copper contains about 105 90% of the original silver. The liquor is next treated with  $\text{H}_2\text{S}$ , in a tower 18, to precipitate any traces of zinc and other metals not precipitated by iron. It then goes through thickener 19, and clarifying filter 20, 110 when it is ready to pass to the electrolytic iron cells, except that 5% of the whole is discarded at each cycle and goes to the agitator 21, where enough milk of lime is added to precipitate all of the iron, magnesia, and alumina, as hydrates, at the same time making calcium chloride in solution. The resulting liquor is a water-clear solution containing 115 12% to 14%  $\text{CaCl}_2$ , and goes back to agitator 14, as above mentioned, after separation from the precipitate in thickener 22, and filter 23. The hydrate cake from this filter is waste and contains all the magnesia and alumina dissolved from the original concentrates, as well as about .3 pounds of iron per 120 pound of original copper.

The electrolyte goes to storage tank 24, and thence passes through heater 25 and is delivered to electrolytic diaphragm cell 26, at 125 a temperature of  $70^\circ$  to  $80^\circ$  C. The anolyte 130

from the cell goes back directly to the agitator 1. The surplus, or circulating, catholyte goes through thickener 27, where hydrochloric acid is added in sufficient amount to restore the hydrogen ion concentration to .003 to .005 N. The under flow passes to filter 28, the cake of which passes back to agitator 1, the filtrate returning to 24. The overflow goes through clarifying filter 29 and back to 24. The iron cathodes produced in the cell 26 contain over 99.9% iron, and are ready for the market, or for further treatment. The iron produced is about 1.75 pounds per pound of original copper in the concentrates.

Fig. 2 illustrates an alternative method of chloridizing by roasting instead of by the addition of the calcium chloride solution, as above described. By this method the calcines from roaster 9 will contain about one and one-half times as much sulphur as copper. They are then mixed in a pug mill 30, with all or a portion of the  $\text{CaCl}_2$  solution, made as above described in agitator 21, together with the necessary amount of new  $\text{CaCl}_2$  to make up chlorine losses. The material from the pug mill is delivered to any suitable form of chloridizing roaster 31. The gases from the roaster are condensed in a water scrubbing tower 32. The calcines go to an agitator 33, where they are leached with the tower liquors from 32, and if desired, with a portion of the above-mentioned  $\text{CaCl}_2$  solution not used in 30; and also, if desired, with a portion of return anolyte leach from the electrolytic iron cells. The addition of free chlorine in any desired form into agitator 33, as for example, in the form of bleaching powder, will facilitate the extraction of the gold.

The tails from agitator 33 are dewatered and washed in the usual manner, and the pregnant liquor is then treated for precipitation of gold and silver, on copper in any usual manner; and copper and lead, if present, are precipitated on iron.

It will be seen that virtually the only distinction between the flow of sheets of Fig. 1 and Fig. 2 is that, whereas in the former chloridizing is accomplished in the wet way with  $\text{CaCl}_2$ , in the latter chloridizing is performed in a furnace, also with  $\text{CaCl}_2$ .

An advantage of the flow sheet of Fig. 2, if any, over Fig. 1, lies in the complete extraction of the silver and gold and lead, if present, as well as the copper, from any type of sulphide ore. As already explained, the tails from agitator 10, Fig. 1, contain practically all of the gold, and about 10% to 15% of the silver, and have to be treated further for recovery of these values. One method would be to so conduct the roasting operation in 9 that enough sulphur would remain with these tails to make them susceptible to chlo-

ridizing roasting. They could then be put through the chloridizing roast in precisely the same manner as just described for the cinders from 9, with resulting complete extraction of silver and gold.

My process, as described with either of its modifications, is fully cyclic with reference to chlorine, there being neither loss nor accumulation of this element in the cycle, and at the same time the concentration of magnesia, alumina, and lime, together with zinc, manganese, and other relatively electro-positive elements, is maintained at a standard condition. Furthermore, this is done cheaply, lime and sulphur being the only chemicals required; but these are recovered in the form of artificial gypsum, which is a saleable by-product. By first using a ferric chloride leach upon the raw ore or concentrates with solution of 85% to 90% copper, and then roasting the residue, I obtain the copper remaining insoluble after the chloride leach, in completely soluble form in sulphuric acid, and then by chloridizing the sulfate solution with calcium chloride I convert all the metals to chlorides before sending the solution on to the electrolytic iron cells, and precipitate the lime out of the solution as gypsum. I obtain the major portion of the calcium chloride used for chloridizing by treating the discarded portion of the electrolyte with lime, the balance being fresh calcium chloride added to compensate for loss of chlorine.

If desired, I may chloridize by calcium chloride in a chloridizing roast instead of by the wet way, thus making substantially all the gold and silver soluble in ferric chloride or other chloride leaches.

The described process is applicable to almost any sulphide mineral or combination of same, except that I prefer to keep the zinc content of the original ore or concentrate as low as possible, inasmuch as zinc is removed by  $\text{H}_2\text{S}$ . It is also preferable to treat concentrates rather than ores, because in the latter the content of magnesia, alumina, and other objectionable elements may be so great as to require an excessively large discard of electrolyte at each cycle. It is also preferable that all the minerals treated be in the form of sulphides. Most of the so-called oxidized ores of the metals will be soluble in the combined chloride and sulfate leaches; but these ores should be either eliminated entirely or tolerated in the charge only in small amounts, because they are not as suitable for the cyclic process as are the sulphide minerals.

Having described my process, I claim as my invention:

1. A cyclic metallurgical process for extracting metals from ores containing iron and copper and recovery of same, which consists in subjecting the ore to the leaching

action of a solution of ferric chloride, oxidizing the tails from said leach by roasting, extracting the resulting cinders to yield the copper and portion of iron and other metals as sulfates, chloridizing the sulfate liquor by addition of calcium chloride, treating the pregnant liquors with metallic iron, discarding a portion of the leach, and treating this portion with lime to produce calcium chloride, and electrolyzing the remaining solution containing principally ferrous chloride to produce electrolytic iron and ferric chloride for the chloride leach.

2. A cyclic process of extracting metallic values from ores containing sulphides of iron and/or copper and concentrates containing iron and copper, which consists of subjecting the ores or concentrates to the leaching action of a solution of ferric chloride, oxidizing the tails from said leach by roasting, then extracting from the resulting concentrates the metals in the form of sulphates, converting the metals to chlorides by chloridization of the sulphate solution with calcium chloride, precipitating the calcium sulphate and electrolyzing the remaining solution to produce electrolytic iron and ferric chloride for the leach.

3. In a cyclic process of extracting metallic values from ores containing sulphides of iron and copper, wherein the ores or concentrates are dissolved in ferric salts and the ferrous solution is electrolyzed to bring about a regeneration of ferric salts and the electrolytic deposition of iron, the steps of converting the metals to chlorides by chloridization of the sulphate solution with calcium chloride and obtaining the major proportion of the calcium chloride used for chloridization by treating a portion of the electrolyte with lime and precipitating the lime out of this solution in the form of an artificial gypsum.

4. In a cyclic process for treating sulphide ores containing iron and other metals for recovery of electrolytic iron and other metals, leaching the ore with a solution containing ferric chloride, roasting tails from this leach, dissolving metals from tails as sulphates, converting said sulphates to chlorides, treating all the resulting liquors for precipitation of substantially all metals except iron, electrolyzing the resulting solution for the production of electrolytic iron and the regeneration of the ferric leach.

5. In a process for treating sulphide ores containing iron and copper for recovery of their metallic content, the steps for effecting solution of the metals which consist in first leaching the unroasted ore with a leach containing ferric iron and substantially no acid; and then roasting the residue from this leach and dissolving the remaining metals as sulfates.

6. In a cyclic process for treating sulphide

ores for recovery of their metallic content with the use of separate chloride and sulphate leaching liquors, the step of chloridizing the sulphate liquors after leaching by the addition of calcium chloride.

7. In a cyclic process for treating sulphide ores for recovery of their metallic content with the use of separate chloride and sulphate leaching liquors, the step of chloridizing the sulphate liquors after leaching by the addition of calcium chloride, and making calcium chloride by treating a portion of the chloride liquors after leaching with milk of lime.

8. In a cyclic process for treating sulphide ores for recovery of their metallic content with the use of separate chloride and sulphate leaching liquors, the steps of chloridizing the sulphate liquors after leaching, and adding calcium chloride to the said sulphate liquors to supply chlorine to compensate for losses.

ROBERT D. PIKE.

70

75

80

85

90

95

100

105

110

115

120

125

130